

Patented June 14, 1927.

1,632,456

# UNITED STATES PATENT OFFICE.

CHARLES SWAN, OF LONG BEACH, CALIFORNIA.

METHOD OF FORMING PAVING COMPOSITIONS.

No Drawing.

Application filed August 17, 1925. Serial No. 50,853.

My present invention relates to concrete compositions for pavements, sidewalks and the like, which contain a bituminous binder other than the substantially solid bitumen referred to in my Patent No. 1,519,560, granted December 16, 1924; and my present invention relates more particularly to asphaltic paving compositions containing, in suitable admixture with diatomaceous earth, such asphaltic materials as are commonly found in California and other Western States, as also in Central and South American countries, and elsewhere.

It is an object of this invention to provide improved asphaltic paving compositions utilizing naturally fluent asphalts or asphalt fractions, and requiring no use of Trinidad asphalt, or other solid asphaltic ingredients; and it is a further object of my invention to provide an improved method of preparing the novel compositions herein described, or analogous compositions.

As in the case of the prior patent mentioned, I attribute the meritorious qualities of my novel paving compositions mainly to a skillful and judicious proportioning and incorporation of diatomaceous earth; and my former opinion in this regard is confirmed by the facility with which compositions comparable in their properties with those described in my mentioned patent may be prepared, even without the use of solid bitumens, provided the constituent materials, including a viscous or liquid asphalt, but not necessarily including any crude petroleum distinct therefrom, are treated and associated in substantially the manner hereinafter described.

As heretofore mentioned, I have discovered that diatomaceous earth, when used in proper proportions, and treated in a manner favorable to the utilization of its natural properties, not only causes a pavement containing the same to remain substantially unaffected by temperature changes, but also exhibits cementitious properties in the amalgamation of concrete, toughening the pavement and rendering it more elastic and durable. Depending, however, upon the climate in which the composition is to be used, the diatomaceous earth must be suitably proportioned relatively to the asphaltic material with which it is, in the process herein described, initially associated in a fluent material adapted to be admixed, while hot, with an aggregate material also

preheated; and it is an important feature of the novel process herein described that the diatomaceous earth is first separately preheated, when used without additions of crude oil such as are mentioned in my patent above referred to, to a temperature far above the boiling point of water,—even such as a temperature in excess of 1200° F., to facilitate the subdivision of the diatomaceous earth and the separation of clay therefrom.

Other features and advantages of my invention, in the practice of which the proportion of diatomaceous earth may be so varied as to adapt the resultant composition to use either in a tropical or in a cold climate, may be best understood from the following description of an advantageous procedure in the preparation of a paving composition suitable for use in, for example, the climate of southern California:

I may initially preheat a suitable quantity of an asphaltic composition, such as a composition showing a penetration of .40 to .75 (as compared with a penetration of about .35, in the case of Trinidad asphalt—the test here referred to being executed at about 77° F., using a No. 2 needle, a weight of 100 grams, a period of 5 seconds, and proceeding in accordance with the course approved by the American Society for Testing Materials, at its 1916 annual meeting) to a temperature such as 300° to 350° F., more or less; and into this preheated asphalt I may incorporate (as by mixing the same in an agitator having, for example, a capacity of 50 barrels and for a period such as 1½ to 2 hours) from 5% to 35% by weight of diatomaceous earth, previously heated to a temperature such as 600° F., more or less.

When the paving composition into which the described mixture is incorporated is to be used in a climate such as that of Los Angeles, California, 10 to 15 pounds of diatomaceous earth may advantageously be thus initially associated with each 85 pounds of preheated asphalt; and after this mixture has been agitated for a period sufficient to render the same substantially homogeneous, the temperature being kept above 300° F., I may add 6% to 15% of the same to 85%—94% of a suitable aggregate, as an aggregate containing sharp sand and hard gravel in graduated sizes and suitable proportions,—the dry mixture of aggregate materials having been also brought to a temperature above 300° F.

Assuming that both the asphaltic-diatomaceous fluent mixtures are at temperatures between 300° and 400° F. at the time of their association in a suitable mixer, agitation for a period such as 10 minutes may be sufficient to incorporate the same in such manner as to permit immediate use; and it will be understood to be necessary to lay and roll or otherwise compact the composition 10 before its temperature shall drop below about 180° F.

Any temperature between about 180° F. and 250° F. is suitable to the rolling and finishing of a pavement containing the 15 scribed composition,—which should, of course, be laid upon a dry and solid base, preferably to a thickness not less than 1 inch, the top surface being either finished in a general manner described in my men- 20 tioned patent or by the application of a seal coat of hot asphalt uniformly squeegeed over the surface at the rate of from .2 to .3 gallon per square yard. After the squeegee coat has been applied, hot screening may be 25 broadcasted over the surface, in the case of a pavement intended for vehicular use, and rolled until fairly bonded to the road, additional screening being optionally spread and broomed over the surface, during roll- 30 ing, in sufficient quantity to take up all excess asphalt.

In explanation of my reference to the use of comparatively high temperatures in conditioning the diatomaceous earth, I may 35 mention that temperatures greatly in excess of the boiling point of water are, if at all, used, primarily to facilitate the separation of foreign matter such as clay, present as an impurity in most commercial diatomaceous earth. Temperatures above 3000° F. 40 must be avoided as tending to break up the diatom skeletal units, and temperatures as low as 600° F., or less, may be sufficient in the case the heating is done in blower tube, the 45 clay being caught on a screen through which the diatoms pass. When a rotary furnace is used, a satisfactory purification of the diatomaceous earth may be favored by a temperature even above 2000° F. the clay tending to collect at a lower level but being 50 removable by, for example, a tilting of the furnace. In any case, originally pure or purified diatomaceous earth may be permitted to cool to about the temperature of the hot asphalt before it is admixed therewith.

Relative proportions of coarse and fine aggregate, and the maximum sizes tolerated, 55 may naturally depend upon the thickness of the pavement; and the proportion of diatomaceous earth initially associated with fluent asphalt, after suitable preheating of both of these ingredients, may vary from, for example, 20% of diatomaceous earth 60 with 80% of asphalt, when my composition

is to be used in a torrid climate such as that of the Imperial Valley, California, to proportions such as 5% of diatomaceous earth used with 95% of fluent asphalt, when the composition is to be used in a cooler climate 70 such as that of Seattle, Washington,—8% being suggested as suitable for use in San Francisco, and 10% to 15% being suitable for use in Los Angeles. It will, however, be understood that all figures given herein 75 are merely illustrative of the principles and practice of my invention, numerous additions and modifications being possible, without the slightest departure from the spirit and scope of my invention, as the same is 80 indicated above and in the following claims.

I claim as my invention:

1. A method of forming paving compositions which comprises: separately preheat- 85 ing naturally fluent asphalt, showing a penetra- 90 tion of about .40 to .75 under conditions which result in a penetration of only about .35 in the case of Trinidad asphalt, and diatomaceous earth to temperatures about 300° F., the diatomaceous earth being heated to a 95 higher temperature than the asphalt and incorporated therewith in proportion between 5% and 35%; separately preheating an aggregate mixture to a temperature above 300° F.; and mixing the resultant asphaltic-di- 100 atomaceous earth mixture with said aggregate mixture at an elevated temperature.

2. A method of forming paving compositions which comprises: separately preheat- 100 ing naturally fluent asphalt, showing a penetra- 105 tion of about .40 to .75 under conditions which result in a penetration of only about .35 in the case of Trinidad asphalt, and diatomaceous earth to temperatures above 300° F., the diatomaceous earth being heated to a 110 higher temperature than the asphalt and incorporated therewith in proportions between 5% and 35%; separately preheating an aggregate mixture to a temperature above 300° F.; and mixing the resultant asphaltic diatomaceous earth mixture with said aggregate mixture at an elevated temperature, said diatomaceous earth, when containing foreign matter, being first preheated to a temperature between 600° F. and 115 3000° F.

3. A method of forming paving compositions which comprises: separately preheat- 120 ing naturally fluent asphalt, showing a penetra- 125 tion of about .40 to .75 under conditions which result in penetration of only about .35 in the case of Trinidad asphalt, and diatomaceous earth to an elevated tempera- 130 ture, the diatomaceous earth being heated to a higher temperature than the asphalt, the diatomaceous earth and the described naturally fluent asphalt being mixed at an elevated temperature in proportions between 5% of diatomaceous earth with 95% of asphalt and 35% of diatomaceous earth 135

with 65% of asphalt by weight, separately preheating an aggregate mixture to a temperature above 300° F.; and mixing the resultant asphaltic-diatomaceous earth mixture with said aggregate mixture at an elevated temperature.

4. A method of forming paving compositions which comprises: separately preheating naturally fluent asphalt and diatoma-

ceous earth to temperatures above 300° F., 10 higher temperature than the asphalt and incorporated therewith in proportions between 5% and 35%.

In testimony whereof, I have hereunto set my hand at Los Angeles, California, this 12th day of August, 1925.

CHARLES SWAN.